

## UNITED STATES PATENT OFFICE.

JOHN P. ARNOLD, OF COLFAX, ILLINOIS.

## EXPLOSIVE COMPOUND.

SPECIFICATION forming part of Letter Patent No. 757,713, dated April 19, 1904.

Application filed October 18, 1902. Serial No. 127,812. (No specimens.)

*To all whom it may concern:*

Be it known that I, JOHN P. ARNOLD, a resident of Colfax, in the county of McLean and State of Illinois, have invented certain new and useful Improvements in Explosive Compounds, of which the following is a specification.

This invention relates to improvements in explosive compounds and method of making the same, and refers more specifically to the production of an improved smokeless or semi-smokeless gunpowder well adapted for use in small firearms and for analogous purposes.

The object of my invention is to provide an explosive which may be readily ignited, which burns uniformly and rapidly, thereby imparting a high rate of speed to the projectile or charge and with a minimum amount of recoil; to provide a compound which is not objectionably sensitive to moisture and not seriously affected thereby within reasonable limits; to provide a compound which burns with the production of a minimum amount of visible smoke and which fouls the chamber of the firearm to a minimum degree; to provide a compound the ingredients of which are of relatively low cost and which is mixed or compounded in an extremely simple and economical manner, and in general to provide an improved explosive compound of the character referred to.

The invention consists in the matters hereinafter described, and more particularly pointed out in the appended claims.

My improved explosive consists of chlorate of potash, yellow prussiate of potash, saltpeter, sulfur, and tannin, or the equivalents of these ingredients, which, according to my improved method, are compounded or mixed as follows: To make one hundred pounds of powder I take chlorate of potash, forty-nine pounds; yellow prussiate of potash, thirty pounds; saltpeter, ten pounds; sulfur, five pounds; tannin, six pounds. These several ingredients I finely pulverize separately in any suitable and usual manner and then mix the ingredients while dry. The ingredients are then mixed with about five gallons of a liquid which is a solvent of the tannin and is not a solvent of the other ingredients. Al-

cohol is such a solvent. Preferably I employ wood-alcohol of that kind commonly known as "Columbian spirits." The ingredients having been mixed with the alcohol, I preferably boil the mixture from two to five minutes in a suitable vessel and thereafter cool and drain the composition and allow it to dry into a plastic mass of the proper consistency to be granulated by passing it through a suitable granulating-screen. The mixture is then granulated by passing through a screen and thereafter thoroughly dried.

Instead of boiling the mixture I may extend the treatment over a greater length of time and reach the same end—namely, the dissolving and thorough distribution of the tannin without the employment of heat—that is to say, the tannin is soluble in alcohol without heating the latter—and the thorough distribution of the tannin may be accomplished by mechanically agitating or mixing instead of by ebullition.

The tannin referred to as forming one of the ingredients is preferably ordinary commercial tannic acid. In place of common salt-peter (nitrate of potash) I may use as an alternative nitrate of soda, (Chili salt-peter,) and the term "salt-peter" used in the claims is intended to include both. The tannin may be supplied in any one of the forms of tannic acid or tannins. That step of the process which consists in treating the ingredients in a solvent of the tannin is an important feature or step in securing the desired results, it being found that the powder so produced possesses greater power, burns more uniformly and rapidly, and is less susceptible to moisture. It is believed that the solvent acts to dissolve the tannin and insures that each particle of the several ingredients is thoroughly covered or coated with tannin and that this results in an improved composition and product. At any rate it has been demonstrated that the treatment of the ingredients in a solvent in the manner described substantially improves the character of the compound, although it is probable that no substantial quantity of the alcohol remains in the powder after the latter has been granulated and thoroughly dried.

A powder compounded in accordance with my invention is entirely safe to handle, ignites very readily, and is practically smokeless when used in firearms. Moreover, it is not substantially affected by ordinary atmospheric conditions, and even though it becomes relatively damp it ignites and burns freely while in this condition. Its rate of combustion is relatively high or rapid, and the explosion is accompanied by the minimum amount of recoil.

While I have herein described what I deem to be the preferred proportions of the several ingredients, yet it will of course be understood that these proportions may be to a certain extent varied without departing from the invention.

I claim as my invention—

1. An explosive compound, consisting of

chlorate of potash, yellow prussiate of potash, salt peter, sulfur and tannin, substantially as herein described.

2. An explosive compound consisting of chlorate of potash, yellow prussiate of potash, salt peter, sulfur and tannin, the tannin existing in the compound in the form of a binder adherent to the non-soluble substances.

3. An explosive compound consisting of chlorate of potash, yellow prussiate of potash, salt peter, sulfur and tannin, the tannin existing in the compound as a coating of the insoluble ingredients, brought to this condition by being dissolved in alcohol, and the latter evaporated out, substantially as described.

JOHN P. ARNOLD.

Witnesses:

ALBERT H. GRAVES,  
L. F. McCREA.